

## UNITED STATES PATENT OFFICE

2,274,657

## ALUMINUM ALLOY

Walter Bonsack, South Euclid, Ohio, assignor to  
 The National Smelting Company, Cleveland,  
 Ohio, a corporation of Ohio

No Drawing. Application April 17, 1941,  
 Serial No. 389,019

2 Claims. (Cl. 75—146)

This invention relates to alloys, and particularly to aluminum base alloys having high strength at ordinary and elevated temperatures and being suitable for casting, working and heat treating.

It is an object of this invention to produce alloys having relatively high elongation and relatively high tensile strength.

It is a further object of this invention to provide a relatively light alloy which may be easily cast and machined, which may be used at elevated temperatures without a rapid deterioration in the desirable properties, and which may be readily treated with anodic treatment to give excellent lustre and finish.

It is a still further object of this invention to provide an alloy having a relatively high proportional limit and a relatively high fatigue strength, and in which these properties may be further enhanced by heat treatment.

In my copending application Serial No. 284,527, filed July 14, 1939, of which this application is a continuation-in-part, I have described an aluminum alloy containing magnesium and zinc in the proportions to form, with part of the aluminum, a ternary compound of aluminum, magnesium and zinc. When magnesium and zinc are added to aluminum in the proper proportions, a ternary compound of aluminum, magnesium and zinc is formed, which compound may be in solid solution in the aluminum. The ternary compound improves the characteristics of aluminum, giving the alloy high strength combined with relatively high ductility, good color and excellent corrosion resistance.

The casting properties of such an alloy may be greatly improved, however, by the presence of silicon in an amount more than an impurity. In an alloy containing sufficient magnesium to combine with all the silicon, silicon does not exist as free silicon, but avidly combines with the magnesium to form magnesium silicide ( $Mg_2Si$ ), which compound improves the casting properties.

In calculating the amount of magnesium and zinc that should be present in the aluminum alloy to form the desired percentage of ternary compound, the magnesium which is not used up in combining with the silicon is to be considered as that available for combination with the zinc and a portion of the aluminum to form the ternary compound. Therefore, in making the alloy one should first determine the amount of magnesium silicide desired before calculating the total amount of magnesium that should be present in

the alloy to form the desired amount of ternary compound.

The ternary compound is said by some investigators to have a composition having substantially the formula  $Al_3Mg_7Zn_6$ , and other investigators have considered the formula for the ternary compound as being  $Al_2Mg_3Zn_3$ . It will be seen that the amounts of magnesium and zinc relative to each other are quite similar in both formulas and, for the purposes of the improved alloy, the magnesium and zinc should be present in about the proportion necessary to form the ternary compound of either formula.

An excess of zinc, over and above that which cooperates with magnesium and aluminum to form a ternary compound according to the above formula having the greatest proportion of zinc, increases the brittleness and decreases the ductility of the alloy. Also, it tends to cause a decline in the ultimate strength and proportional limit. For this reason it is undesirable that zinc be present in quantities substantially greater than the amount sufficient to react to form such a ternary compound with magnesium and aluminum. The most desirable properties are obtained when the magnesium and zinc are proportioned so that the ratio of magnesium (uncombined with any silicon) to zinc is about equal to the ratio represented by the formula  $Al_2Mg_3Zn_3$ , or somewhat larger, as represented by the formula  $Al_3Mg_7Zn_6$ . It is usually desirable to have the magnesium present on the rich side to prevent the silicon from being in excess and taking magnesium away from the ternary compound.

Magnesium adds to the hardness and machining qualities of the alloy and, as above stated, should be present in an amount sufficient to combine with the available silicon to form the ternary compound with the zinc and aluminum present. A small amount of magnesium may be provided to replenish losses that may occur when the alloy metal is remelted. In greater quantities magnesium tends to make the alloy sluggish, decreasing castability.

Magnesium and zinc have heretofore been added to aluminum in the proportion represented by about the formula  $MgZn_2$ . It has been found, however, that a given percentage of ternary compound is more effective in producing desirable properties and, because the zinc content of the ternary alloy is less, they have a lower density.

The improved aluminum alloys of this invention may have the ternary compound of aluminum, zinc and magnesium present in an amount ranging from about 1% to about 8%. But, with

the preferred alloys, the zinc and the magnesium uncombined with the silicon are proportioned to form about 2% to about 6% of the ternary compound, with possibly a small amount of magnesium uncombined with the silicon and the ternary compound  $Al_3Mg_7Zn_8$ . At room temperature the ternary compound is present in solid solution in aluminum alloys in an amount of about 2%. The percentage in solid solution increases at high temperatures and decreases upon cooling, the excess precipitating out. Aluminum alloys containing the ternary compound may, therefore, be advantageously heat treated to improve their properties.

Magnesium silicide in small proportions may be present in aluminum alloys containing sufficient magnesium to react with the silicon present as an impurity. While the magnesium-silicide equivalent to such a quantity of silicon may slightly improve the casting properties of alloys containing the ternary compound of aluminum, magnesium and zinc, it has been found that such ternary alloys having more magnesium silicide, preferably between about 3% and about 5%, have their casting properties considerably improved. As much as 8% magnesium silicide may be present in the alloys, however. Calcium combines even more avidly with silicon than magnesium, and its silicide, in small amounts, may be substituted for part of the magnesium silicide. Calcium silicide supplements the magnesium compound without materially affecting the properties of the alloy. When calcium silicide is also present, the total silicide should preferably be between about 3% and 8%.

In forming the alloys of the present invention the magnesium should, therefore, be present in sufficient amount to combine with the free silicon, or that uncombined with any calcium, to form  $Mg_2Si$  and in addition to combine with the zinc to form the ternary compound according to the formula  $Al_2Mg_3Zn_3$ , the formula requiring the least magnesium relative to the zinc.

2% or 3% of the ternary compound of aluminum, magnesium and zinc improves the properties of aluminum or aluminum alloys, and such alloys may be cast. The casting properties, however, are usually also improved when the alloy contains more of the ternary compound than 2% or 3%. An increase in strength and a decrease in elongation are ordinarily obtained with increased quantities of the ternary compound.

The presence of the ternary compound of aluminum, magnesium and zinc in aluminum base alloys is quite advantageous in producing alloys having relatively high tensile strength, relatively high proportional limit, relatively high fatigue, and relatively high elongation, even at somewhat elevated temperatures, and which alloys may have their properties further improved by heat treatment. As before explained, the ternary compound is particularly of advantage in aluminum base alloys having a relatively low silicon content, such as less than 1.5%.

The percentages of zinc and magnesium in the ternary compound are almost the same, regardless of which of the above mentioned formulae are considered the basis for the computation. Thus, in each percentage of the ternary, on the basis of the formula  $Al_3Mg_7Zn_8$  there is about .26% magnesium and about .5% zinc, and on the basis of the formula  $Al_2Mg_3Zn_3$  there is about .22% magnesium and about .6% zinc.

About 1.75% magnesium is required to combine with each percent of uncombined silicon to form

magnesium silicide ( $Mg_2Si$ ) before any ternary compound will be formed. For example, if 1% of the ternary compound on the basis of  $Al_2Mg_3Zn_3$  be desired in an alloy having 1% silicon, the amount of magnesium to be added to form the ternary compound will be about .22%, and the magnesium to combine with 1% silicon will be about 1.75%, making a total of about 2%.

The magnesium and zinc to provide for 2% of the ternary  $Al_2Mg_3Zn_3$  in an alloy having 1% free silicon or about 3%  $Mg_2Si$  would be about 2.25% magnesium and 1.2% zinc. Similarly, with such an allowance the magnesium and zinc for an alloy containing 3% free silicon or about 8%  $Mg_2Si$  and 8%  $Al_2Mg_3Zn_3$  would be about 7% or 8% and 4.8% respectively.

In the alloys of the present invention, zinc should be present in amounts from about .6% to about 4.8%, and preferably from 1.2% to about 3.6%. The magnesium should be present within the limits of about 2% and about 8%, and preferably between about 2% and 5.5% or 6%, depending on the amount of zinc and silicon in the alloy. Magnesium silicide should be present in amounts of 3% to 8%, and preferably between 3% and about 5%. The amount of magnesium uncombined with silicon should be proportioned to the zinc to form with the zinc and part of the aluminum a ternary compound of aluminum, magnesium and zinc. Additional magnesium should also be present to combine with the silicon to form magnesium silicide, and to provide an excess, such as .5%. That is, for the formation of the ternary compounds and the improved alloys of the present invention, the magnesium is related to the zinc and silicon and is about 35% to 45% of the zinc plus 1.75% of the silicon content.

The aluminum alloys of the present invention containing magnesium, uncombined with silicon, and zinc in the proportion of a ternary compound, when cast in molds of a design such that chilling takes place substantially simultaneously in the various portions of the casting, form good castings without the use of grain refining agents. However, it has been found that certain grain refining elements substantially improve the properties of the aluminum alloy containing the ternary compound.

The grain refiners which I have found improve the properties of the alloy are members of the group consisting of boron in the amount of .005% to 1%, zirconium in the amount of .01% to .5%, tungsten in the amount of .01% to .5%, molybdenum in the amount of .01% to .5%, vanadium in the amount of .01% to .5%, titanium in the amount of .05% to .5%, columbium in the amount of .01% to .5% and tantalum in the amount of .05% to .5%. These grain refining elements should preferably be present in a total amount of from .005% to .5%, and it is frequently desirable to have more than one of these elements present in a given alloy.

While the grain refiners in the above group are desirable in the alloys of the present invention, not all of the grain refiners affect the properties in the same way. The particular refiner or group of refiners selected in any given instance depends on the particular condition which must be satisfied. The grain refiners selected from the group consisting of titanium, tungsten, molybdenum, zirconium and vanadium, and especially tungsten and molybdenum, improve the strength and the elongation of the castings. Of these, titanium, being less expensive, is usually used

for ordinary castings, but in cases where the highest elongation, together with strength, is necessary, it is preferred to use tungsten or molybdenum. The grain refiners selected from the group consisting of boron, columbium and tantalum do not appear to appreciably increase the strength or elongation of the alloy and are usually used where appearance, finish and corrosion resistance are most important and where strength is of less consequence. Certain grain refiners, such as cerium, were found to be relatively undesirable in the alloy.

The above described hardening elements, manganese, chromium, nickel and copper, substantially decrease the hot shortness, improve the properties of the alloy, and assist in maintaining the improved properties at high temperatures, such as are encountered in internal combustion engines. The above grain refining elements, particularly members of the group consisting of tungsten, molybdenum, vanadium and titanium, also have this property when present in substantial amounts, such as .2% or .3%, or so. It is, therefore, especially desirable to have up to .5% or so of these latter elements present when the hardening ingredients are absent.

An aluminum base alloy containing about 3% magnesium silicide ( $Mg_2Si$ ), magnesium and zinc in the proportion to form with the aluminum about 6% of the ternary compound  $Al_3Mg_7Zn_4$ , and .2% titanium was chill cast into test bars. The best bars were quenched from the mold and aged for seven days at room temperature, and, when tested, showed a tensile strength of 38,000 lbs./sq. in., a yield strength of 28,300 lbs./sq. in., a proportional limit of 21,500 lbs./sq. in., and an elongation of 2.1%. The titanium may be substituted by another grain refiner selected from the above group, but when the grain refiner was omitted the strength was somewhat reduced.

Test bars of the above alloy were air cooled and aged for seven days. When tested they showed a tensile strength of 37,100 lbs./sq. in., a yield strength of 28,800 lbs./sq. in., a proportional limit of 21,000 lbs./sq. in., and an elongation of 1.6%.

An alloy having the same constituents as the above alloy, except that only about 1.5% magnesium silicide was present, was chill cast into test bars which were quenched and aged as above. While the test bars thus prepared had a tensile

strength slightly higher than those shown above, the proportional limit was 19,000 lbs./sq. in., the yield strength was 26,000 lbs./sq. in., and the elongation was 4.3%. This alloy also was not quite as readily castable.

The alloys disclosed herein have good fatigue and tensile strengths, and a relatively high proportional limit, even at relatively high temperatures; they may be heat treated to improve and modify their properties; and they have sufficient ductility and hardness so that they can be used as structural shapes, castings, machine parts, etc. These alloys have a desirable color, high corrosion resistance, and may be anodically finished or highly polished with excellent results.

It is to be understood that the particular compounds disclosed and the procedure set forth are presented for purposes of explanation and illustration, and that various equivalents can be used and modifications of said procedure can be made without departing from my invention as defined in the appended claims.

What I claim is:

1. An aluminum base alloy of relatively high strength and ductility, comprising magnesium, zinc, magnesium silicide, one or more metals for hardening or grain refining, and the balance substantially all aluminum and minor impurities, the zinc being present in the amount of about .6% to 4.8%, the magnesium silicide being present in the amount of about 3% to 8%, the amount of magnesium in the alloy uncombined with silicon being about 35% to 45% of the zinc content, the total magnesium being within the range of about 2% to 8%, and the total silicon being within the range of about 1% to 3%.

2. An aluminum base alloy of relatively high strength and ductility, comprising magnesium, zinc, magnesium silicide, one or more metals for hardening or grain refining, and the balance substantially all aluminum and minor impurities, the zinc being present in the amount of about 1.2% to 3.6%, the magnesium silicide being present in the amount of about 3% to 5%, the amount of magnesium in the alloy uncombined with silicon being about 35% to 45% of the zinc content, the total magnesium being within the range of about 2% to 5.5%, and the total silicon being within the range of about 1% to 2%.